

## UNITED STATES PATENT OFFICE

1,952,575

## COLLET STEEL

Douglas G. Anderson, Elmira, N. Y.

No Drawing. Application December 11, 1931,  
Serial No. 580,508

3 Claims. (Cl. 75—1)

The object of my invention is to produce an alloy steel particularly suited to the manufacture of certain machine elements requiring a high degree of hardness and resilience. For example 5 my improved steel may be used to advantage in the manufacture of collets and feed fingers for automatic lathes or screw machines.

Taking as an example the manufacture of collets, it is necessary that the steel used for this 10 purpose should develop great hardness in the bore of the collet to withstand abrasion from the rod clamped therein. At the same time the steel must be sufficiently resilient to return to its original shape after being released from compression in the spindle head or chuck. It must also 15 withstand the drastic internal stresses set up when the collet is hardened without cracking. This is a difficult requirement to meet since sharp corners, slots and sudden changes in cross section cannot be avoided in the design of collets 20 and since the maximum hardness (and hence the most drastic quenching action) is required in the slotted end of the bore where these undesirable features are concentrated.

25 It has heretofore been common practice to use a carbon or carbon-vanadium tool steel in the manufacture of collets and to water quench the collet after it has been machined. Steels of this type may for example contain:

|           | Percent     |
|-----------|-------------|
| Carbon    | .95 to 1.05 |
| Manganese | .20 to .30  |
| Silicon   | .15 to .25  |
| Vanadium  | .15 to .25  |

35 While collets made of this steel and water quenched are in general sufficiently hard and resilient, it has proved difficult to produce the more complicated types (particularly those with wide variations in cross section) without breakage in 40 hardening.

As is well known in the art of heat treating, it is often possible to avoid breakage in hardening by substituting oil for water in the quenching operation. As a rule, however, simple carbon 45 or carbon-vanadium steels do not develop their maximum hardness when quenched in oil and I have found that collets made of these steels and oil quenched are not sufficiently hard to be satisfactory in service. Furthermore, the so-called 50 alloy tool steels containing chromium as the principal hardening agent and which are commonly oil quenched have not proved to be sufficiently resilient for satisfactory collets. These steels are also considerably more expensive than simple 55 carbon steels or my improved collet steel.

I have found that if the content of manganese in a steel of the carbon or carbon-vanadium type is increased from the usual range, say .20 to .40%, to about .80%, that the resulting steel when oil quenched will develop the desirable hardness and 60 resiliency of the water quenched carbon steel; and that oil quenching practically eliminates the danger of breakage. The compositions which I have found most suitable for this purpose lie 65 within the following range:

|           | Percent  |
|-----------|----------|
| Carbon    | .80—1.50 |
| Manganese | .60—.90  |
| Silicon   | .20—.40  |
| Vanadium  | .10—.30  |
|           | 70       |

It is to be understood that my invention resides in the use of a relatively high content of manganese which permits satisfactory oil hardening of a composition otherwise requiring water quenching. The above analysis ranges may therefore be expanded considerably without departing from the spirit of my invention. As in the case of other steels, it may be necessary, for example, to vary the carbon content through a considerable range in order to adjust the hardening properties of the steel to the section to be hardened. Vanadium in amounts up to .30% may or may not be used in my steel as desired. When present, vanadium exerts its usual cleansing and toughening effect upon the steel.

Having thus described my invention what I claim as new and desire to secure by Letters Patent is:

1. An oil hardening tool steel composed of iron, from about .80% to about 1.10% of carbon, from about .60% to about .90% of manganese and from about .15% to about .25% of vanadium.
2. An oil hardened article made from steel composed of iron, from about .80% to about 1.10% of carbon, from about .60% to about .90% of 95 manganese and from about .15% to about .25% of vanadium.
3. An oil hardened collet made from steel composed of iron, from about .80% to about 1.10% of carbon, from about .60% to about .90% of manganese and from about .15% to about .25% of vanadium.

DOUGLAS G. ANDERSON.

105

110